

June 11, 1935.

J. A. WEIGER

2,004,259

VALVE SEAT

Filed Oct. 22, 1931



Fig. 1



Fig. 3



Fig. 2



Fig. 4

Fig. 5



INVENTOR

BY Joseph A. Weiger  
Watson, Bristol, Johnson, Leavenworth  
ATTORNEYS

## UNITED STATES PATENT OFFICE

2,004,259

## VALVE SEAT

Joseph A. Weiger, Indianapolis, Ind., assignor to  
 P. R. Mallory & Co., Incorporated, Indianapolis,  
 Ind., a corporation of Indiana

Application October 22, 1931, Serial No. 570,339

6 Claims. (CL 123—188)

This invention relates to valve seats, and more particularly to valve seats for use in internal combustion engines.

5 A general object of the invention is the provision of an improved valve seat which is admirably suited to withstand the deteriorating conditions encountered at the ports of an internal combustion engine, and particularly at the exhaust ports thereof.

10 More specifically, the invention has for objects the provision of a valve seat having enhanced heat resisting properties which will not anneal at operating temperatures, will not tend to pit or transfer metal to the cooperating valve part, 15 is susceptible to machining, has a proper coefficient of thermal expansion to assure a tight fit with the cylinder block under operating conditions, and has an extremely long service life as compared to other materials.

20 Other objects of the invention will in part be obvious and will in part appear hereinafter.

The invention accordingly comprises a product possessing the features, properties, and the relation of components which will be exemplified 25 in the product hereinafter described and the scope of the application of which will be indicated in the claims.

For a fuller understanding of the nature and objects of the invention reference should be had 30 to the following detailed description taken in connection with the accompanying drawing, in which:

Fig. 1 is a plan view showing one form of valve seat embodying features of the present invention;

Fig. 2 is a transverse sectional view taken on a diameter of the seat shown in Fig. 1;

Fig. 3 is a plan view showing a modified form of valve seat;

40 Fig. 4 is a transverse sectional view taken on a diameter of the seat shown in Fig. 3; and

Fig. 5 is a fragmentary sectional view taken through a portion of an engine cylinder block showing, on a reduced scale, the valve seat of 45 Fig. 1 inserted in place therein.

In accordance with the present invention, it has been found that generally enhanced characteristics can be imparted to valve seats which are designed for use in internal combustion engines by using in their formation a metallic body comprising, in its preferred form, tungsten which has been treated with a hardening agent, such as carbon, and cemented or impregnated with a relatively low melting point material such as 55 copper. Such material is particularly well suited

successfully to withstand the deteriorating conditions encountered at the exhaust ports of such an engine. A material of this kind is disclosed in a co-pending application of George N. Sieger and Joseph A. Weiger, Serial No. 52,690, which has matured into Patent No. 1,848,437, and does not, per se, form any part of the present invention, except insofar as it is utilized in connection with valve seats which are subjected to deteriorating influences such as those encountered in internal combustion engines. A composite valve seat formed by inserting the herein contemplated improved metallic material in a metallic seat member is described and claimed in my co-pending application, Serial No. 570,338. The seats there shown are more particularly suited for use with valves of large size, and may be manufactured more economically than rings formed entirely of the herein described hard metallic material. The invention claimed in this application refers to valve seats formed in toto of this material. Such a ring is well adapted for use with smaller sizes of valves, where the amount of material required to form a complete seat is relatively limited. It is, of course, also applicable to valves of larger size, and no limitation as to size is intended in the present description and claims.

The material from which it is here proposed to make valve seats may be formed in several ways. The preferred method of forming a hard metallic valve seat material comprises forming a porous slug of refractory metal, treating with a hardening agent, sintering and impregnating it with a fused low melting point metal. Such a 35 slug may be obtained by mixing powdered tungsten and carbon, pressing the mixture to shape, and sintering it; or powdered tungsten may be pressed into form and sintered in a carbonaceous atmosphere. The slug thereafter may be immersed in or subjected to fused copper, which will run throughout the porous structure, the impregnation being abetted by capillary action.

For the purposes of the present invention, tungsten is a preferred refractory metal, although other similar metals in the same group and subgroup of Mendelejeff's periodic table, such as molybdenum, which may in some cases prove satisfactory, are contemplated. The hardening agent preferably is carbon, in the form of lamp black, although other hardening materials for the refractory metal may be used, wherefore no specific limitation is intended. The hardening agent may be present in any desired amount, but preferably is present in an amount 50 55

less than the combining weight thereof with the amount of refractory metal used. When carbon and tungsten are used, for example, the preferred amount of the carbon is less than that 5 needed to convert all the tungsten into a carbide, whereby the tungsten becomes partially carburized upon heating, but does not lose its identity. Carbides of tungsten are, among other things, more difficult to machine than the preferred product. Copper is a preferred low melting point metal, although any metals having proper characteristics as to fusion point, corrosion resistance, mechanical strength, and the like, are contemplated. Silver, for example, is 10 a suitable cementing material where the operating temperatures to which the valve seat is subjected do not run too high. The heating is preferably carried out in a reducing, neutral or carburizing atmosphere, such as, for example, hydrogen, nitrogen, or hydrocarbon atmosphere. 15

While the ingredients and proportions used in the present valve seat are subject to variations within reasonable limits, a preferred form of material embodying the invention is given by 20 way of example as follows:

|          | Percent |
|----------|---------|
| Tungsten | 80      |
| Carbon   | 0.3     |
| Copper   | 19.7    |

30 A cemented, sintered body made from these ingredients, in accordance with the above outline, or any other suitable methods, is remarkably suited for its intended function as a valve seat.

35 Referring more particularly to the drawing, and especially to Figs. 1 and 2 thereof, there is shown a centrally perforate seat member 11, having its upper internal margin bevelled to an angle 40 of approximately 45°, as illustrated at 12, to provide a seating surface for cooperation with the valve head. This valve seat is formed of the herein described hard cemented or impregnated tungstic material. The finely divided ingredients used in the manufacture of this material 45 may be pressed in a ring shaped mold, in order to give the ultimately formed product substantially its proper shape. After a ring of such cemented or impregnated tungsten-carbon-copper has been formed, it is suitably machined.

50 In Figs. 3 and 4, there is shown a somewhat different form of valve seat which also is formed of the herein contemplated hard tungstic composition. This seat comprises a ring 21, having in Fig. 4, the flat upper face 22 of which is adapted to provide the wearing surface. The powdered materials used in the formation of this type of ring may be pressed into form in a ring shaped 55 mold, as in the case of the preceding embodiment, after which they likewise are heat treated in a hydrogen atmosphere, in order to sinter and harden the tungstic base and fuse the low melting point metal, which is adapted to cement or impregnate such base.

55 In each of the modifications shown, after the ring is removed from the heat treating furnace, it is necessary to machine at least the inside diameter and one face of the valve seat. The 60 material used in the present ring, while possessing the proper hardness, strength, and non-corrosive qualities to assure an extremely long and satisfactory service life, has good machining properties and may be readily ground and lapped.

70 75 These grinding and lapping operations ordinarily

will take place after the valve seat has been fitted to the cylinder block, to assure a proper cooperating fit between the valve head and seat.

The described forms of seats made from this material are admirably suited for shrink-fitting to the cylinder block of an engine. The block, which usually is made of cast iron, may be locally heated and the valve seat dropped into place. If preferred, the seat may be cooled, for example, by immersion in liquid air, and 10 dropped into place in the cylinder block. Upon return to room temperature, a tight fit is secured, it being possible even to obtain a slight dovetail fit between the parts. The valve seat of the herein contemplated improved material is shown 15 thus fitted to a cast iron cylinder block in Fig. 5. The coefficient of thermal expansion of the improved hard metal composition is such as admirably to suit it to these shrink-fitting operations, and also to preserve a tight fit between 20 the valve seat and cylinder block under operating conditions. In addition, this composition has proper heat resisting qualities and will not anneal during engine operation, nor will it pit or transfer metal to the cooperating valve part. 25

Coupled with these desirable qualities, it has extremely long service life as compared with other materials. No previously used valve seat material of which applicant is aware has the long life, coupled with good machining qualities, proper coefficient of thermal expansion, corrosion resistance and heat resistance properties which 30 characterize the herein described product.

35 Although, in many of the following claims, tungsten is recited as one of the ingredients utilized in the contemplated improved valve seat metal, it will readily be apparent from the foregoing description that other compatible elements, for example molybdenum, may be used in lieu thereof, or in combination therewith. Accordingly, it is intended that the recital of tungsten 40 as an element in these claims shall be construed to refer not only specifically to that element, but also to other equivalent elements and particularly to those which are herein mentioned. 45

It will be seen that there has been disclosed a valve seat which is admirably suited to fulfill its intended functions.

50 Since certain changes may be made in the above product and different embodiments of the invention could be made without departing from the scope thereof, it is intended that all matter contained in the above description or shown in the accompanying drawing shall be interpreted as illustrative and not in a limiting sense. 55

It is also to be understood that the following claims are intended to cover all of the generic and specific features of the invention herein described, and all statements of the scope of the invention which, as a matter of language, might 60 be said to fall therebetween.

Particularly, it is to be understood that in said claims, ingredients or compounds recited in the singular are intended to include compatible mixtures of such ingredients wherever the sense permits.

Having described my invention, what I claim as new and desire to secure by Letters Patent, is:

1. A valve seat for internal combustion engines, 70 formed of a cemented metallic body comprising approximately four-fifths of a refractory metallic element chosen from the group and sub-group of Mendelejeff's periodic table of elements which includes tungsten, a metal of a lower melting point incorporated therewith, and a 75

- harden ing agent present in an amount less than the combining weight thereof with the quantity of tungsten present.
2. A valve seat for internal combustion engines, formed of a cemented metallic body comprising a porous base of tungsten in preponderating amount, and carbon in an amount sufficient to harden said base, and copper impregnating said porous base.
- 5 3. A valve seat for internal combustion engines, formed of a cemented metallic body comprising approximately four-fifths tungsten forming a porous base, copper incorporated in the pores of said base, and carbon in an amount less than the combining weight thereof with the amount of tungsten used to form a carbide of tungsten.
4. A valve seat for internal combustion engines, formed of a porous partially carburized tungsten base and copper impregnating said porous base.
- 5 5. A valve seat for internal combustion engines, formed of a sintered metallic body consisting of approximately 80 per cent tungsten, 19.7 per cent copper and 0.3 per cent carbon.
6. A valve seat for internal combustion engines, comprising a ring of porous partially carburized, sintered tungsten and copper incorporated in the pores thereof.
- 10 JOSEPH A. WEIGER. 15